# EUROPEAN PATENT SPECIFICATION

(11) **EP 2 217 736 B1**
(45) Date of publication and mention of the grant of the patent: **27.03.2019**
(21) Application number: 07870514.2
(22) Date of filing: 26.10.2007
(51) Int. Cl.: C23C 4/08, C23C 4/18, C23C 4/02

(54) **A PROCESS FOR PRODUCING BODY CENTERED CUBIC (B2) NICKEL ALUMINIDE (NIAL) COATING OF CONTROLLED THICKNESS ON NICKEL-BASE ALLOY SURFACES**
VERFAHREN ZUR HERSTELLUNG EINER BESCHICHTUNG AUS KUBISCH-RAUMZENTRIERTEM (B2) NICKELALUMINID (NIAL) MIT KONTROLLIERTER DICKE AUF NICKELBASISLEGIERUNGSOBERFLÄCHEN
PROCÉDÉ DE PRODUCTION D'UN REVÊTEMENT D'ALUMINURE DE NICKEL (NIAL) À STRUCTURE CUBIQUE CENTRÉE (B2) D'ÉPAISSEUR CONTRÔLÉE SUR DES SURFACES D'ALLIAGE À BASE DE NICKEL

(43) Date of publication of application: 18.08.2010
(73) Proprietor: The Secretary, Department Of Atomic Energy, Govt. of India, Mumbai 400 001, Maharastra (IN)
(72) Inventor: GANESAN, Srinivasan, Kalpakkam (IN); BHADURI, Arun Kumar, Tamilnadu 603102 (IN); RAJ, Baldev, Tamilnadu 603102 (IN); VENKATRAMAN, Gopal, Tamilnadu 600028 (IN)
(74) Representative: Fresh IP
(86) International application number: PCT/IN2007/000514
(87) International publication number: WO 2009/053992

(56) References cited:
- EP-A- 0 985 745
- EP-A- 1 254 967
- US-A- 3 000 755
- US-A- 3 129 069
- US-A- 3 450 512
- US-A- 4 501 776

## Description

### FIELD OF THE INVENTION

The present invention relates to aluminizing of nickel-base alloys and, in particular, to a process for producing body centered cubic (B2) nickel aluminide (NiAl) coating of controlled thickness using thermal spraying of commercially pure aluminium wires followed by diffusion heat treatment in vacuum atmosphere on nickel-base alloys surfaces. Importantly, the process of producing the nickel aluminide (B2 NiAl phase) coatings on nickel-base alloys is directed to achieve dimensional tolerance of 80 ± 30 microns coating thickness.

Advantageously, the process of the invention achieves nickel aluminide coatings only on desired regions of the substrate of the nickel base alloys with minimum environmental emission of toxic chemicals fumes and is thus also environment friendly. Moreover, the nickel aluminide coating of the present invention is possible without the need for masking of the unwanted regions of the components and more importantly can be attended both on flat and curved surfaces thereby favouring wide scale utilities of such aluminizing process. The process of the invention would facilitate fabrication industries required to carry out surface modifications and engineering (protective coating) on nickel-base alloys for high temperatures such as nuclear industries, aircraft and gas turbine industries.

### BACKGROUND ART

It is well known that nickel-base alloys are required to be provided surface modified and engineered for protective coatings such as wear resistance, oxidation resistance, corrosion resistance etc., to adopt such nickel-base alloys for high temperature application for variety of industrial and allied uses.

Aluminizing on nickel-base alloys is usually known to be carried out by processes such as pack cementations, slurry spraying, brushing, dipping and chemical vapour deposition to produce nickel aluminide (NiAl) layer over the substrate adapted for providing a hard surface for fretting wear and galling resistance.

It also known to carry out thermal spray processes alone for deposition of metals on worn out surfaces of steel components. Also, it is well known to achieve pack diffusion and vapour phase diffusion coatings for protection against wear and fretting of fast reactor components. Aluminium paint - based processes for producing NiAl coating have also been used previously. While, the above existing state of the art prevails for the nickel aluminide coating on nickel base alloys there has been some inherent limitations/disadvantages of such hitherto known processes and devices.

Pack cementations is a process which has been widely used for such aluminizing since it is inexpensive and ideally suited for batch production of small components. In such pack cementation process, the components to be aluminized are usually treated at temperatures between 850°C and 1050°C in a pack consisting of an aluminium source such as Ni-AI, Ti-Al, or Cr-AI, an activator (halide) and some inert filler like alumina. It is however, experienced that such pack cementation technology involves handling of large quantities of alumina and metal powders, long furnace time cycles due to a large thermal inertia and inherently reduced throughput.

Vapour phase aluminizing on the other hand largely eliminates the disadvantages of the pack cementation processes, but required specialized vacuum furnaces and fixtures. Moreover, both these processes involve exposure of operator to corrosive halide activators which is unsafe and undesired from the safety of the operator.

US 3,000,755 is directed to oxidation-resistant turbine buckets and nozzle guide vanes for gas turbine engines. More particularly, the same is concerned with nickel base alloy and cobalt base alloy turbine buckets having surfaces provided with a protective layer of an alloy of the base metal with aluminium wherein a portion of the coating metal is diffused into the base metal to thereby form with the base metal an oxidant-resistant surface layer of an alloy of the coating metal and said base metal having a thickness not in excess of 63.5 µm (0.0025 inch).

US 3,129,069 is again directed to oxidation resistant turbine buckets and nozzle guide vanes for gas turbine engines. More particularly, the patent suggests an alloy of aluminium with the base metal of blade having a thickness of approximately 12.7 µm (0.0005 inch).

US 3450512 refers to a method for applying aluminum- tungsten coating on nickel base alloys. This patent is primarily directed to prevent the inter-diffusion between the base metal and the coating materials whereby the mixture of aluminum and tungsten are metalized of the alloy surface and the 4 hour long post metallization diffusion heat treatment is carried out to form a nickel-aluminum alloy, nickel-aluminide (NiAl) at the surface of the article and distribute the tungsten in solid solution and metallurgically bond the coating to the substrate.

However while the above prior art proposed possible Nickel aluminide coating none of the above prior arts were either directed to or even hinted at aluminizing methods for producing surface protective coating of B2 phase (Body centered cubic) NiAl layer/coating of desired controlled thickness on nickel-base alloy surfaces through an inter-diffusion between coated aluminum and nickel of the alloy surfaces.

Apart from the above discussed limitations and complexities of the conventional methods of aluminizing on nickel-base alloys to achieve B2 phase (Body centered cubic NiAl) layer/coating, it is also important that following such processes of aluminizing it has been always essential to mask the surfaces which were not required to be coated requiring special precautions and added complexities of such aluminizing processes.

### OBJECTS OF THE INVENTION

It is thus the basic object of the present invention to provide for a process for NiAl aluminide coating in particular the B2 phase (Body centered cubic NiAl) layer/coating of controlled thickness on nickel-base alloys using thermal spraying of commercially pure aluminium wires followed by diffusion heat treatment in vacuum atmosphere as a surface modification and engineering protective coating for application of fretting wear and galling resistance of the nickel-base alloy substrate.

Another object of the present invention is directed to a process for NiAl aluminide coating in particular the B2 phase (Body centered cubic NiAl) layer/coating of nickel-base alloys which would on one hand be cost effective and at the same time on the other hand would involve safe technology without the problems/disadvantages of handling of large quantity of alumina and metal powder, long furnace time cycle due to large thermal inertia and inherent reduced throughput.

Further object of the present invention is directed to a simple process for NiAl aluminide coating in particular the B2 phase (Body centered cubic NiAl) layer/coating of nickel-base alloys which would also not require any specialized vacuum furnaces and fixtures and thus can be readily applied and used for producing nickel aluminide coatings.

A further object of the present invention is directed to an aluminizing process which would favour achieving NiAl aluminide coating in particular the B2 phase (Body centered cubic NiAl) layer/coating on nickel-base alloys to a tolerance of 80 ± 30 µm with reduced cycle time than the conventional pack cementation and vapour phase diffusion coating.

Yet another object of the present invention is directed to favour production of body centered cubic (B2) nickel aluminide (NiAl) coated nickel-base alloys of controlled thickness without the complexities of masking of surfaces not to be coated thereby facilitating controlled and simple production of such nickel aluminide coated nickel-base alloys.

A further object of the present invention is to produce ordered body centered cubic (B2) nickel aluminide (NiAl) coated nickel-base alloys which can be advantageously used to form the coating only on the desired regions without any special steps to masking the areas where aluminizing is not desired.

Yet another object of the present invention is directed to produce ordered body centered cubic (B2) nickel aluminide (NiAl) coated nickel-base alloys with higher productivity, environmental cleanliness and suitability for mass production of large sized components.

Yet another object of the present invention is directed to a process which would achieve NiAl aluminide coating in particular the B2 phase (Body centered cubic NiAl) layer/coating on nickel-base alloys involving flat and/or corrugated surfaces to thereby favour production of variety of NiAl aluminide coated nickel-base alloys.

A further object of the present invention is directed to produce surface protective coating in particular the B2 phase (Body centered cubic NiAl) layer/coating for high temperature application to improve the wear resistance of the substrate on nickel-base alloys with selectively controlled coating thickness which can be consistently reproduced.

Yet further object of the present invention is to provide for a simple yet effective process for producing surface protective coating in particular the B2 phase (Body centered cubic NiAl) layer/coating for high temperature application on nickel-base alloys which would favour overall reduction of time and cost for aluminizing vis-à-vis the conventional processes of aluminizing of such nickel-base alloys presently in use.

### SUMMARY OF THE INVENTION

Thus according to the basic aspect of the present invention there is provided an aluminizing process for producing surface protective body centered cubic (B2) nickel aluminide (NiAl) coating of controlled thickness of 80 µm with tolerance of 30 µm on nickel-base alloy surfaces with minimum 40 weight % nickel content comprising:
activating the surfaces to be coated by grit blasting involving alumina grit with 30-120 mesh size at an air pressure of 5.5+/-0.5 kg/cm² preferably following dimensional check and degreasing;
thermal spraying of the required surfaces with commercial pure aluminium to desired specific thickness in the range of 100 to 200 µm wherein thermal spray parameters comprise (i) aluminum wire diameter in the range of 3.0 to 3.2 mm at a wire Feed Rate in the range of 2.0-2.5mm/sec (ii) pneumatic pressure in the range of 5.5+/-0.5 kg/cm² (iii) oxygen pressure in the range of 2.5+/-0.3 kg/cm² and acetylene pressure in the range of 1.0+/-0.2 kg/cm² and (iv) maintaining a torch work distance of 200-300 mm;
subjecting the aluminium thus sprayed onto the nickel-base alloy substrate to diffusion heat treatment in vacuum atmosphere at a temperature in the range of 950°C-1100°C for a duration of 1.0 to 1.5 hours such that the sprayed aluminium reacts with the nickel-base alloy substrate to form the desired nickel aluminide coating of said controlled thickness on the nickel-base alloy substrate; and
subjecting the coated surface to surface cleaning.

Preferably, in the above aluminizing process for producing surface protective coating of body centered cubic (B2) nickel aluminide (NiAl) coating, the surface cleaning of the coated surface comprise removing adherent oxide scale using pickling solution following the steps of:
(i) providing the pickling solution preferably comprising (a) concentrated nitric acid (specific gravity :1.41 g/cm³) in amounts of 16% (by volume);(b) Hydrofluoric acid (specific gravity 1.61 g/cm³) in amounts of 3.5 % (by volume); and (c) Water in amounts of 80.5% (by volume);
(ii) soaking the diffusion treated strips in the solution for a period of about 30 minutes; followed by
(iii) further cleaning the strips involving emery papers.

Following the above disclosed aluminizing process for producing surface protective coating of body centered cubic (B2) nickel aluminide (NiAl) coating of the invention it is possible to carry out the NiAl aluminide coating on nickel-base alloys involving selectively flat and/or corrugated surfaces.

The above disclosed aluminizing process for producing surface protective coating of body centered cubic (B2) nickel aluminide (NiAl) of the invention is four times higher than conventional process of aluminizing nickel-base alloy.

Importantly, in the above process the surface activity, spraying procedures and diffusion parameters are critical in optimization of the coating thickness. Surface activity is achieved by selection of suitable grade grit size (30-120 mesh size) during grit blasting. Thermal spraying of aluminium is carried out using 3.2 mm diameter aluminium wires and by maintaining a torch-work distance of 200-300 mm and wire feed rate of 2.0-2.5 mm/sec. Thickness of sprayed layer is monitored on 100% of the qualification strips and on a certain percentage of production strips at random to ensure sprayed layer thickness of 100-200 µm. The optimized diffusion treatment is carried out in a vacuum furnace at 950-1100°C for 1.0-1.5h.

It is thus possible by way of the present invention discussed above to produce ordered body centered cubic (B2) nickel aluminide (NiAl) coating of controlled thickness on nickel-base alloys involving a selective thermal spray-diffusion process. Importantly, the process of the invention achieves selective advantages in producing such coated nickel-base alloys by involving the thermal spraying which is a process in which molten or semi-molten particles are applied by impact on to the surface at uniform rate using mechanise or manually operated spray gun.

The selective diffusion treatment after thermal spray in vacuum atmosphere is involved whereby the aluminium melts and reacts with the nickel/iron base alloys to thereby form the desired B2 phase.

Importantly, the major advantage in the above process of the invention involving the combination of thermal spraying and diffusion treatment is that the same avoids the complexities of masking of uncoated surfaces and yet can favour achieving the coating only on the desired surfaces of the nickel-base alloys. This is an important advantage in the present process of producing the nickel aluminide coated nickel-base alloys of the invention since the conventional coating process of such alloys such as the conventional pack cementation process, hot-dip process etc., essentially required coating the entire strip unless special steps are taken to mask the area where aluminizing is not desired.

The process being simple to operate and apply favours for higher productivity and is importantly environment friendly and safe from the operators point of view since the same does not require the operator to be exposed to corrosive environment such as corrosive halide activators involved in the conventional pack cementation and vapour phase aluminizing processes.

The details of the invention, its object and advantages are explained hereunder in greater detail in relation to non-limiting exemplary illustration of the process of the invention as per the following accompanying figure and examples :-

### BRIEF DESCRIPTION OF THE ACCOMPANYING FIGURE:

Figure 1: is a schematic illustration of the stages involved in the aluminizing of Ni-base alloys in accordance with the present invention involving thermal spray and diffusion treatment.

As shown in said figure the basic steps involved in such process of aluminizing comprises of carrying out sequentially (a) dimensional checks, (b) degreasing, (c) grit blasting, (d) thermal spraying, (e) diffusion treatment, (f) surface finish and (g) dimensional check. Such a process of aluminizing involving the thermal spray and diffusion treatment of the invention is illustrated further by way of the following example.

### EXAMPLE

An Exemplary process of aluminizing of nickel-base alloys following the process of the invention involving the thermal spraying and diffusion treatment was carried out as detailed hereunder:
i) The nickel-base alloys surface to be coated was first activated ,after dimensional check and degreasing , by grit blasting using alumina grit of specific size and size distribution i.e., in the range of 30-120 mesh size at a air pressure of 5.5 ± 0.5 kg/cm²;
ii) thereafter thermal spraying of the required surfaces using commercially pure aluminium (dia 3.2 mm) to specific thickness in the range 100 to 200 microns was carried out using the following thermal spray parameters thermal spray parameters:
   a) wire feed rate : 2.0 - 2.5 mm/sec.;
   b) pneumatic pressure: 5.5±0.5 kg/cm²;
   c) oxygen pressure: 2.5 ± 0.3 kg/cm²; and
   d) acetylene pressure : 1.0 ± 0.2 kg/cm².
iii) subsequently diffusion heat treatment was carried out in vacuum atmosphere at specified temperature in the range 950 - 1100°C for a duration of 1.0-1.5 h to enable the aluminium sprayed to react with the nickel - iron - chromium alloys substrate and form the aluminide coating;
iv) subsequently surface cleaning procedure was carried out to remove adherent oxide scale using a pickling solution as per the following details :
   a) concentrated nitric acid (specific gravity : 1.41 g/cm³) : 16% (by volume);
   b) hydrofluoric acid (specific gravity 1.61 g/cm³): 3.5 % (by volume);and
   c) water: 80.5% (by volume).
The pickling solution obtained as above was used to soak the diffusion treated strips for 30 minutes followed by hand cleaning of the strips such as by using 400 grit size emery papers.

By way of the above disclosed process of the invention it was possible to produce the ordered body centered cubic (B2) nickel aluminide (NiAl) coating of controlled thickness on nickel-base alloys involving the simple yet effective thermal spray-diffusion process.

Advantageously, the present aluminizing process can achieve NiAl aluminide coating on nickel-base alloys with minimum 40 wt% nickel content on both flat and corrugated surfaces. Moreover, the processes found suitable for mass production of large sized components to a tolerance of 80± 30 µm of NiAl aluminide coating with hardness range of 800 - 1100 VHN with reduced cycle time as compared to the conventional processes such as the pack cementation and vapour phase diffusion coating. Moreover, the process of the invention involving the selective combination of thermal spray and diffusion heat treatment would favour coating on selected areas of the components both on flat and curved surfaces without the need for masking and its related complexities. Thus, the process offers overall reduction of time and cost of aluminizing which is found to be four time faster than the conventional processes of aluminizing nickel-base alloys.

The present process would thus enable producing surface protective coatings for high temperature applications to improve the wear resistance on nickel-base alloys with controlled coating thickness which importantly can be consistently reproduced. Moreover, the process would favour the desired surface areas alone to be aluminized without the need for complex masking of uncoated areas. The process offers overall reduction of time and cost for aluminizing. The duration of aluminizing for other conventional processes is four times higher than the present invention and the process would therefore favour much simpler and faster generation of NiAl coated Ni-base alloys both on flat and/or corrugated surfaces apart from being environment friendly and safe to carry out.

## Claims

1. An aluminizing process for producing surface protective coating of body centered cubic (B2) nickel aluminide (NiAl) of controlled thickness of 80 µm with tolerance of 30 µm on nickel-base alloy surfaces with minimum 40 weight % nickel content comprising:
activating the surfaces to be coated by grit blasting involving alumina grit with 30-120 mesh size at an air pressure of 5.5+/-0.5 kg/cm² preferably following dimensional check and degreasing;
thermal spraying of the required surfaces with commercial pure aluminium to desired specific thickness in the range of 100 to 200 µm wherein thermal spray parameters comprise (i) aluminum wire diameter in the range of 3.0 to 3.2 mm at a wire Feed Rate in the range of 2.0-2.5mm/sec (ii) pneumatic pressure in the range of 5.5+/-0.5 kg/cm² (iii) oxygen pressure in the range of 2.5+/-0.3 kg/cm² and acetylene pressure in the range of 1.0+/-0.2 kg/cm² and (iv) maintaining a torch work distance of 200-300 mm;
subjecting the aluminium thus sprayed onto the nickel-base alloy substrate to diffusion heat treatment in vacuum atmosphere at a temperature in the range of 950°C-1100°C for a duration of 1.0 to 1.5 hours such that the aluminium sprayed reacts with the nickel-base alloy substrate to form the desired nickel aluminide coating of said controlled thickness on said nickel-base alloy substrate; and
subjecting the coated surface to surface cleaning.

2. An aluminizing process for producing surface protective coating of body centered cubic (B2) nickel aluminide (NiAl) according to claim 1 wherein the said surface cleaning of the coated surface comprise removing adherent oxide scale using pickling solution following the steps of:
(i) providing the pickling solution preferably comprising (a) concentrated nitric acid (specific gravity :1.41 g/cm³) in amounts of 16% (by volume);(b) Hydrofluoric acid (specific gravity 1.61 g/cm³) in amounts of 3.5 % (by volume); and (c) Water in amounts of 80.5% (by volume);
(ii) soaking the diffusion treated strips in the solution for a period of 30 minutes; followed by
(iii) further cleaning the strips involving emery paper.

3. An aluminizing process for producing surface protective coating of body centered cubic (B2) nickel aluminide (NiAl) according claim 1 or 2 wherein the NiAl aluminide coating is carried out on nickel-base alloys involving selectively flat and/or corrugated surfaces.

4. An aluminizing process for producing surface protective coating of body centered cubic (B2) nickel aluminide (NiAl) according to anyone of claims 1 to 3 wherein the aluminizing process is four times higher than conventional process of aluminizing nickel-base alloy.

## Patentansprüche

1. Aluminisierungsverfahren zur Produktion einer Oberflächenschutzbeschichtung aus raumzentriertem kubischem (B2) Nickelaluminid (NiAl) mit einer kontrollierten Dicke von 80 µm mit einer Toleranz von 30 µm auf Oberflächen aus einer Legierung auf Nickelbasis mit einem Nickelgehalt von mindestens 40 Gew.-%, umfassend:
Aktivieren der zu beschichtenden Oberflächen durch Sandstrahlen, das Aluminiumoxid-Strahlsand beinhaltet, mit einer Maschenweite von 30-120 bei einem Luftdruck von 5,5 +/- 0,5 kg/cm², vorzugsweise nach Maßprüfung und Entfettung;
thermisches Spritzen der erforderlichen Oberflächen mit gewerblichem reinem Aluminium auf eine gewünschte spezifische Dicke im Bereich von 100 bis 200 µm, wobei thermische Spritzparameter (i) einen Aluminiumdrahtdurchmesser im Bereich von 3,0 bis 3,2 mm bei einer Drahtvorschubgeschwindigkeit im Bereich von 2,0-2,5 mm/s, (ii) einen Druckluftdruck im Bereich von 5,5 +/- 0,5 kg/cm², (iii) einen Sauerstoffdruck im Bereich von 2,5 +/- 0,3 kg/cm² und einen Acetylendruck im Bereich von 1,0 +/- 0,2 kg/cm² und (iv) ein Aufrechterhalten eines Brennerarbeitsabstands von 200-300 mm umfassen;
Unterziehen des so auf das Substrat aus einer Legierung auf Nickelbasis gespritzten Aluminiums einer Diffusionswärmebehandlung in einer Vakuumatmosphäre bei einer Temperatur im Bereich von 950 °C - 1100 °C für eine Dauer von 1,0 bis 1,5 Stunden, so dass das gespritzte Aluminium mit dem Substrat aus einer Legierung auf Nickelbasis reagiert, um die gewünschte Nickel-Aluminiumbeschichtung mit der kontrollierten Dicke auf dem Substrat aus einer Legierung auf Nickelbasis zu bilden; und
Unterziehen der beschichteten Oberfläche einer Oberflächenreinigung.

2. Aluminisierungsverfahren zur Produktion einer Oberflächenschutzbeschichtung aus raumzentriertem kubischem (B2) Nickelaluminid (NiAl) nach Anspruch 1, wobei die Oberflächenreinigung der beschichteten Oberfläche ein Entfernen von anhaftendem Zunder unter Verwendung einer Beizlösung gemäß den folgenden Schritten umfasst:
(i) Bereitstellen der Beizlösung, die vorzugsweise (a) konzentrierte Salpetersäure (spezifische Dichte: 1,41 g/cm³) in Mengen von 16 % (bezogen auf das Volumen); (b) Fluorwasserstoffsäure (spezifische Dichte: 1,61 g/cm³) in Mengen von 3,5 % (bezogen auf das Volumen) und (c) Wasser in Mengen von 80,5 % (bezogen auf das Volumen) umfasst;
(ii) Eintauchen der diffusionsbehandelten Streifen in der Lösung für einen Zeitraum von 30 Minuten; gefolgt vom
(iii) weiteren Reinigen der Streifen, das Sandpapier beinhaltet.

3. Aluminisierungsverfahren zur Produktion einer Oberflächenschutzbeschichtung aus raumzentriertem kubischem (B2) Nickelaluminid (NiAl) nach Anspruch 1 oder 2, wobei die NiAl-Aluminidbeschichtung auf Legierungen auf Nickelbasis durchgeführt wird, die wahlweise flache und/oder gewellte Oberflächen beinhalten.

4. Aluminisierungsverfahren zur Produktion einer Oberflächenschutzbeschichtung aus raumzentriertem kubischem (B2) Nickelaluminid (NiAl) nach einem der Ansprüche 1 bis 3, wobei das Aluminisierungsverfahren um das Vierfache höher als ein herkömmliches Verfahren zur Aluminisierung einer Legierung auf Nickelbasis ist.

## Revendications

1. Procédé d'aluminisation pour produire une couche de protection superficielle d'aluminure de nickel (NiAl) cubique centrée sur le corps (B2) d'une épaisseur contrôlée de 80 µm, avec une tolérance de 30 µm sur des surfaces d'alliage à base de nickel comprenant une teneur en nickel minimale de 40 % en poids, consistant à :
activer les surfaces devant être revêtues par grenaillage impliquant du grain abrasif à base d'alumine avec une taille de maille de 30-120 à une pression atmosphérique de 5,5+/-0,5 kg/cm², de préférence suite à un contrôle dimensionnel et un dégraissage ;
pulvériser thermiquement des surfaces requises avec de l'aluminium commercial pur jusqu'à une épaisseur spécifique prévue se situant dans la plage de 100 à 200 µm, dans lequel les paramètres de pulvérisation thermique comprennent (i) un diamètre de fil d'aluminium se situant dans la plage de 3,0 à 3,2 mm à une Vitesse d'Avance de Fil se situant dans la plage de 2,0 à 2,5 mm/sec, (ii) une pression pneumatique se situant dans la plage de 5,5+/-0,5 kg/cm², (iii) une pression d'oxygène se situant dans la plage de 2,5+/-0,3 kg/cm² et une pression d'acétylène se situant dans la plage de 1,0+/-0,2 kg/cm² et (iv) le maintien d'une distance de travail à la flamme de 200 à 300 mm ;
soumettre l'aluminium ainsi pulvérisé sur le substrat en alliage à base de nickel à un traitement thermique de diffusion dans une atmosphère sous vide à une température se situant dans la plage de 950 °C à 1100 °C, pendant une durée de 1,0 à 1,5 heure, de sorte que l'aluminium pulvérisé réagisse au substrat d'alliage à base de nickel pour former la couche d'aluminure de nickel souhaitée ayant ladite épaisseur contrôlée sur ledit substrat d'alliage à base de nickel ; et
soumettre la surface revêtue à un nettoyage de surface.

2. Procédé d'aluminisation pour produire une couche de protection superficielle d'aluminure de nickel (NiAl) cubique centrée sur le corps (B2) selon la revendication 1, dans lequel ledit nettoyage de surface de la surface revêtue comporte la suppression de calamine adhérente à l'aide d'une solution de décapage à la suite d'étapes consistant à :
(i) prévoir la solution de décapage comportant de préférence (a) de l'acide nitrique concentré (gravité spécifique : 1,41 g/cm³) en quantités de 16 % (par volume) ; (b) de l'acide hydrofluorique (gravité spécifique : 1,61 g/cm³) en quantités de 3,5 % (par volume), et (c) de l'eau en quantités de 80,5 % (par volume) ;
(ii) tremper les sections traitées de diffusion dans la solution pendant une durée de 30 minutes ; puis
(iii) en outre nettoyer les sections en utilisant du papier émeri.

3. Procédé d'aluminisation pour produire une couche de protection superficielle d'aluminure de nickel (NiAl) cubique centrée sur le corps (B2) selon, soit la revendication 1, soit la revendication 2, dans lequel la couche d'aluminure est effectuée sur des alliages à base de nickel impliquant des surfaces sélectivement plates et/ou ondulées.

4. Procédé d'aluminisation pour produire une couche de protection superficielle d'aluminure de nickel (NiAl) cubique centrée sur le corps (B2), selon l'une quelconque des revendications 1 à 3, dans lequel le procédé d'aluminisation est quatre fois plus élevé qu'un procédé conventionnel d'aluminisation d'alliage à base de nickel.
